

## UNITED STATES PATENT OFFICE.

WILLIAM E. SHEENE, OF BALTIMORE, MARYLAND, ASSIGNOR TO THE NATIONAL ASPHALT BURIAL VAULT COMPANY, OF BALTIMORE, MARYLAND, A CORPORATION.

## ASPHALT-MASTIC AND COAL-TAR-MASTIC CASKET VAULT.

No Drawing.

Application filed November 19, 1921. Serial No. 516,312.

*To all whom it may concern:*

Be it known that I, WILLIAM E. SHEENE, citizen of the United States, residing at Baltimore, and State of Maryland, have invented certain new and useful Improvements in Asphalt-Mastic and Coal-Tar-Mastic Casket Vaults, of which the following is a specification.

This invention is a burial container of the type designed to receive, house and protect a coffin or casket which is to be placed in a grave and thus buried in the earth.

The prime object of the present invention is to provide such a burial container as will be proof against seepage, and will effectually exclude air, water, dampness and any and all destroying agents to which burial containers are subject when buried in the earth.

The container of the present invention is molded from a bituminous mastic (an asphaltic mastic or a coal tar mastic) and I have determined by actual and satisfactory tests that a container made from a bituminous mastic and buried in the earth or submerged in water will possess the above mentioned desirable characteristics, and in addition thereto the mastic can be readily and inexpensively produced and containers molded therefrom in a satisfactory and inexpensive manner.

In carrying out my invention, I first produce the bituminous mastic which preferably comprises bitumen (asphalt or coal tar by-products), limestone dust, fuller's earth, infusorial earth, and it also comprises sand or grits which form a body or filler thereof.

In some instances it is found advisable to add to the above ingredients a material known as asphalt flux. This gives the materials when mixed a higher degree of efficiency.

In preparing the composition, I prefer to use the ingredients in about the following proportions—viz., approximately sixteen (16) per cent of bitumen, thirty-four (34) per cent of limestone dust, fuller's earth, or infusorial earth, and fifty (50) per cent of sand or grits, it being understood, of course, that good results can also be obtained

by varying the materials in other proportions, and also to the above named ingredients there can be added five (5) to seven (7) per cent of asphalt flux, which will increase the efficiency of the composition when mixed.

When using the limestone dust it is not necessary to use fuller's earth or infusorial earth, and vice versa.

All of the ingredients as stated above are mixed together and cooked until said mixed ingredients reach a paste or mortar consistency such as will be capable of being poured into moulds. It is first, cooked at a temperature of about 450° Fahrenheit for approximately four (4) hours, and stirred constantly either by hand or machine. It is then poured into moulds or forms, and when chilled or cooled to a certain degree it assumes the configuration of the moulds or forms, after which time the moulds or forms can be removed.

It is to be understood that the lid for this receptacle is made of the same ingredients, only poured into a different kind of mould, and the lid is sealed to the receptacle by a composition of the same ingredients, cooked in the same manner, with the exception of adding the sand or grits.

The burial container of the present invention is relatively light in weight as compared with containers made of stone or concrete, and is also fireproof and waterproof, and in fact possesses in a high degree all of the desired properties necessary to a burial container for protecting caskets or coffins when buried in the earth.

What I claim as new is:

1. A burial container comprising a molded casing formed from a bituminous mastic including limestone, sand and bitumen.

2. A burial container comprising a molded casing formed from a bituminous mastic including 16 per cent of asphalt, 34 per cent of limestone and 50 per cent of sand.

In testimony whereof I hereunto affix my signature.

WILLIAM E. SHEENE.